# EUROPEAN PATENT SPECIFICATION

(11) **EP 3 085 799 B1**
(45) Date of publication and mention of the grant of the patent: **17.01.2018**
(21) Application number: 16166305.9
(22) Date of filing: 21.04.2016
(51) Int. Cl.: C22C 9/06

(54) **COPPER ALLOY AND METHOD FOR MANUFACTURING THE SAME**
KUPFERLEGIERUNG UND VERFAHREN ZUR HERSTELLUNG DAVON
ALLIAGE DE CUIVRE ET SON PROCÉDÉ DE FABRICATION

(30) Priority: 22.04.2015 JP 2015087888; 29.02.2016 JP 2016037126
(43) Date of publication of application: 26.10.2016
(73) Proprietor: NGK Insulators, Ltd., Nagoya-city, Aichi 467-8530 (JP); Osaka Alloying Works, Co., Ltd., Fukui-shi, Fukui 910-3138 (JP)
(72) Inventor: UDA, Minoru, Nagoya-city, Aichi 467-8530 (JP); ISHIKAWA, Takahiro, Nagoya-city, Aichi 467-8530 (JP); MIZUTA, Taiji, Fukui-city, Fukui 910-3138 (JP); MIZUTA, Yasunari, Fukui-city, Fukui 910-3138 (JP); TANIGUCHI, Hiroyasu, Fukui-city, Fukui 910-3138 (JP)
(74) Representative: Naylor, Matthew John

(56) References cited:
- WO-A1-2008/103688
- JP-A- 2009 242 895

## Description

The present application claims priority from Japanese Patent Application No. 2015-087888 (filed on 22 April 2015), and Japanese Patent Application No. 2016-037126 (filed on 29 February 2016).

### TECHNICAL FIELD

The present invention relates to copper alloys and methods for manufacturing the same.

### BACKGROUND ART

A variety of copper alloys have been devised as high-strength copper alloy used for various types of springs, bearings and the like. For example, PTL 1 discloses a copper alloy that is a Ni-Sn-Cu-based spinodal alloy to which Mn has been added to prevent grain boundary precipitation that may occur in copper alloy cast materials. According to PTL 1, when Cr, Mo, Ti, Co, V, Nb, Zr, Fe, Si or the like is added to this copper alloy, Ni-Sn-Mn, Si or those additive elements form a hard intermetallic compound that crystallizes out in the matrix, thus contributing to the increase of wear resistance and seizure resistance. PTL 2 discloses a copper alloy whose strength is increased without reducing the electric conductivity by adding Cr or Zr to copper, and further in which oxides of Cr or Zr are prevented from being formed by controlling the oxygen content to 60 ppm or less. This patent literature describes a technique for adding carbon to a molten material or a molten metal for reducing the oxygen content. Also, PTL 2 discloses that the strength of this copper alloy is increased by adding Ni, Sn, Ti, Nb or the like to the copper alloy, and that grain coarsening is prevented by adding Ti or Nb.

JP-A-2009-242895 discloses a copper alloy of 5 to 20wt% Ni and 5 to 10wt% Sn, the balance being Cu and inevitable impurities. JP-A-2009-242895 discloses that the copper alloy may additionally contain Mn, Fe, Co, Zn, Si, Mg, Ti, and Zr at ≤1wt%.

### CITATION LIST

### PATENT LITERATURE

PTL 1: JP 08-283889 A
PTL 2: JP 07-54079 A

### DISCLOSURE OF THE INVENTION

Although the copper alloys of PTLs 1 and 2 exhibit increased wear resistance and seizure resistance, and increased strength without reducing electric conductivity, the ductilities thereof are low in some cases. Accordingly, the copper alloy can be cracked, for example, during being worked, or the elongation of the resulting product can be small. A Cu-Ni-Sn-based copper alloy superior in ductility is desirable.

The present invention is intended to solve these problems, and a major object of the invention is to provide a Cu-Ni-Sn-based copper alloy superior in ductility and a method for manufacturing the same.

### Solution to Problem

In order to achieve the major object, the following copper alloy is provided.

The copper alloy of the present invention is as set out in claim 1.

The copper alloy of the present invention is superior in ductility because of the presence therein of appropriate amounts of Ni, Sn, element A (at least one selected from the group consisting of Nb, Zr and Ti), and carbon.

### BRIEF DESCRIPTION OF THE DRAWINGS

Fig. 1 show photographs of the appearances of copper alloys after being subjected to rolling with a grooved roll in Experimental Examples 2, 4, 9 and 12.
Fig. 2 shows an electron micrograph and characteristic X-ray images of the ingot of Experimental Example 6.
Fig. 3 shows electron micrographs and EPMA mapping results of the ingot of Experimental Example 9.
Fig. 4 shows electron micrographs and EPMA mapping results of the sample of Experimental Example 8 after being subjected to hardening heat treatment.
Fig. 5 shows an electron micrograph and EPMA mapping results of the sample of Experimental Example 2 after being subjected to hot rolling (after being fractured).
Fig. 6 shows a photograph of the appearance of a forged product of Experimental Example 19.
Fig. 7 shows a photograph of the appearance of a forged product of Experimental Example 20.
Fig. 8 shows a photograph of the appearance of a forged product of Experimental Example 21.

### EMBODIMENTS FOR CARRYING OUT THE INVENTION

The copper alloy of the present invention contains 5% by mass to 25% by mass of Ni, 5% by mass to 10% by mass of Sn, 0.005% by mass to 0.5% by mass of element A (element A being at least one selected from the group consisting of Nb, Zr and Ti), and 0.005% by mass or more of carbon. In the copper alloy, the mole ratio of the carbon to the element A is 10.0 or less. Alternatively, the copper alloy of the present invention may contain 5% by mass to 25% by mass of Ni, 5% by mass to 10% by mass of Sn, 0.005% by mass to 0.5% by mass of element A (element A being at least one selected from the group consisting of Nb, Zr and Ti), 0.01% by mass to 1% by mass of an additive element (the additive element being at least one selected from the group consisting of Mn, Zn, Mg, Ca, Al, Si, P, and B), and 0.005% by mass or more of carbon. In this copper alloy, the mole ratio of the carbon to the element A may be 10.0 or less, and the balance of the composition of the copper alloy may be Cu and inevitable impurities.

Ni is expected to produce the effect of inducing spinodal decomposition in age-hardening heat treatment subsequent to solution heat treatment, and of thereby increasing the strength of copper alloy. When the Ni content is 5% by mass or more, the strength is more increased; when it is 25% by mass or less, the copper alloy exhibits a high ductility, and decrease in electric conductivity due to the addition of Ni is suppressed. Preferably, the Ni content is more than 10% by mass. A copper alloy containing more than 10% by mass of Ni allows a larger amount of carbon to dissolve in the molten alloy when melted. Thus, such a copper alloy is expected to more efficiently form carbide described later. The Ni content is more preferably 14% by mass to 16% by mass. When Ni content is 14% by mass or more, the copper alloy is expected to more efficiently form carbide; when it is 16% by mass or less, the copper alloy exhibits a further high ductility, and decrease in electric conductivity due to the addition of Ni is further suppressed.

Sn is expected to dissolve in the copper alloy to form solid solution, thereby increasing the strength. When the Sn content is 5% by mass or more, the strength is increased; when it is 10% by mass or less, a Sn enriched phase, which can reduce ductility, is not easily formed. The Sn content is more preferably 7% by mass to 9% by mass. When Sn content is 7% by mass or more, the strength is further increased; when it is 9% by mass or less, formation of Sn enriched phase is further suppressed.

Nb, Zr or Ti added as element A is expected to form a carbide with the carbon in the copper alloy, and thus to prevent elemental carbon from precipitating, or to prevent interstitial carbon from penetrating the alloy to form solid solution. When the element A content is 0.005% by mass or more, the amount of carbon unable to form carbide is not excessively increased; when it is 0.5% by mass or less, the molten metal can be so flowable as to prevent casting defects. The element A content may be, for example, in the range of 0.01% by mass to 0.3% by mass. If element A is Nb, the content thereof may be, for example, in the range of 0.01% by mass to 0.1% by mass. If element A is Zr, the content thereof may be, for example, in the range of 0.03% by mass to 0.3% by mass. If element A is Ti, the content thereof may be, for example, in the range of 0.01% by mass to 0.25% by mass. Although at least part of element A is considered to be present in the form of carbide, element A may be present in a form other than carbide. When element A is present as carbide, the grain size of the carbide may be, for example, in the range of 20 µm or less, or 10 µm or less. If the carbide has an excessively large grain size, it is a concern that the hard carbide is likely to cause the copper alloy to crack therefrom.

Carbon (C) is expected to form a carbide with element A in the alloy. The carbide is effective in reducing the grain size of the alloy. Carbon with a content of 0.005% by mass or more can form so adequate an amount of carbide as helps form primary crystals in solidification of the alloy, thus reducing the grain size of the cast structure, and/or can function to pin dislocation effectively during solution heat treatment subsequent to hot working and thus to suppress the increase in size of the recrystallized grains. The lower limit of the element A content may be, for example, 0.01% by mass or more. The upper limit of the element A content may be, for example, 0.2% by mass or less, or 0.1% by mass or less.

In the copper alloy of the present invention, the mole ratio of carbon to element A, that is, MC/MA mole ratio, is 10.0 or less, where MA (mol) represents the amount by mole of element A and MC (mol) represents the amount by mole of carbon (C). When the MC/MA mole ratio is 10.0 or less, the excess carbon unable to form carbide is prevented from remaining in the alloy, and degradation in hot workability and decrease in ductility can be suppressed. The MC/MA mole ratio may be 9.0 or less, 8.4 or less, or 8.0 or less. The lower limit of the MC/MA mole ratio may be, for example, 0.04 or more, 0.1 or more, or 0.2 or more. Alternatively, MC/MA mole ratio may be 5.2 or less, or in the range of lager than 5.2 to 8.4.

The copper alloy of the present invention may further contain at least one additive element selected from the group consisting of Mn, Zn, Mg, Ca, Al, Si, P, and B. These additive elements, which are dissolved in the copper alloy to form a solid solution, are expected to deoxidize the molten metal or to prevent the grains from increasing in size during solution heat treatment. Mn is more preferred as the additive element. The content of the additive element may be, for example, 1% by mass or less in total. The content of the additive element is preferably in the range of 0.01% by mass to 1% by mass, more preferably in the range of 0.1% by mass to 0.5% by mass, and still more preferably in the range of 0.15% by mass to 0.3% by mass. When the content of the additive element is 0.01% by mass or more, the above-described effects can be satisfactorily produced. An additive element content of more than 1% by mass however does not produce a further effect corresponding to the amount added.

The copper alloy of the present invention may be based on C72700 alloy having a composition of Cu-9% by mass Ni-6% by mass Sn; an alloy having a composition of Cu-21% by mass Ni-5% by mass Sn; or C72900 or C96900 alloy having a composition of Cu-15% by mass Ni-8% by mass Sn. In the above compositions, the content (percent by mass) of each constituent can be in the range of the corresponding value ± 1% by mass.

Preferably, the balance of the composition of the copper alloy of the present invention is Cu and inevitable impurities. For example, the copper alloy of the present invention may contain 5% by mass to 25% by mass of Ni, 5% by mass to 10% by mass of Sn, 0.005% by mass to 0.5% by mass of element A (at least one element selected from the group consisting of Nb, Zr and Ti), 0.005% by mass or more of carbon, and the balance being Cu and inevitable impurities, with a carbon-to-element A mole ratio of 10.0 or less. Alternatively, the composition of the copper alloy of the present invention may contain 5% by mass to 25% by mass of Ni, 5% by mass to 10% by mass of Sn, 0.01% by mass to 1% by mass of any of the above-cited additive elements, 0.005% by mass to 0.5% by mass of element A (at least one element selected from the group consisting of Nb, Zr and Ti), 0.005% by mass or more of carbon, and the balance being copper and inevitable impurities, with a carbon-to-element A mole ratio of 10.0 or less. The inevitable impurities include, for example, Fe or at least one of Pb, Bi, Cd, Sb, S, As, Se, and Te, and the total content of the inevitable impurities is preferably 0.5% by mass or less, more preferably 0.2% by mass or less, and still more preferably 0.1% by mass or less.

The grain size of the copper alloy of the present invention measured by the intercept procedure specified in ASTM E112 is preferably 200 µm or less, more preferably 100 µm or less, and still more preferably 50 µm or less. A smaller grain size leads to a higher ductility. Preferably, the "elongation after fracture" of the copper alloy of the present invention is 10% or more. Preferably, the tensile strength of the copper alloy of the present invention is 915 MPa or more. The copper alloy of the present invention may be in the shape of, for example, a plate, a strip, a line, a bar, a tube, or a block, and may have any other shape.

The copper alloy of the present invention is preferably in a state in which element A and carbon are finely dispersed in the matrix thereof. In this state, element A and carbon may form a carbide, or may form an alloy phase or an intermetallic compound with at least one element of Cu, Ni, and Sn. The copper alloy may be in a solution form that will be subjected to hardening heat treatment. The solution form will undergo spinodal decomposition by hardening heat treatment. Thus the tensile strength of the copper alloy is further increased. The solution form may have a tensile strength of less than 915 MPa.

The copper alloy of the present invention may be prepared in the following manufacturing process. The manufacturing process of the copper alloy may include, for example, (a) melting and casting step, (b) homogenization heat treatment step, (c) hot working step, (d) solution heat treatment step, and (e) hardening heat treatment step. At least one of following steps (b) to (e) may be omitted as long as the manufacturing process includes melting and casting step. Each of the steps will be described below.

### (a) Melting and casting step

In this step, raw materials are melted and subjected to casting. Any substances may be used as the raw materials without particularly limitation as long as a desired composition can be prepared. For the raw materials of Cu, Ni, Sn, and element A (and additive elements), elementary substances of these elements or alloys containing two or more of these elements may be used. For the raw material of carbon, a carbon-containing furnace or crucible or a carbon-containing covering material for the molten metal may be used, and this carbon is used as the raw material of carbon. In this instance, only one of the furnace, crucible, covering material and the like may contain carbon, or two or more of them may contain carbon. The carbon in the furnace, crucible, covering material of molten metal, or the like may be graphite, coke or carbon black. The carbon content in the copper alloy can be adjusted by controlling the type of the furnace or crucible material, the type and amount of the covering material, the contact time with carbon, the temperature of contact with carbon, the contact area with carbon, or the like.

For the melting and casting step, raw materials selected according to the above-described composition of the copper alloy can be used. For example, the raw materials may be selected and used so that the copper alloy can contain 5% by mass to 25% by mass of Ni, 5% by mass to 10% by mass of Sn, 0.005% by mass to 0.5% by mass of element A (element A is at least one selected from the group consisting of Nb, Zr and Ti), 0.005% by mass or more of carbon, and the balance being Cu and inevitable impurities, with a carbon-to-element A mole ratio of 10.0 or less. Also, the raw materials may be selected and used so that the copper alloy can further contain 0.01% by mass to 1% by mass of an additive element (at least one selected from the group consisting of Mn, Zn, Mg, Ca, Al, Si, P, and B). Alternatively, the raw materials are selected and used so that the copper alloy can have a composition containing 14.0% by mass to 16.0% by mass of Ni and 7.0% by mass to 9.0% by mass of Sn. Element A may be Nb, and the raw materials may be selected and used so that the Nb content can be in the range of 0.005% by mass to 0.1% by mass. Element A may be Zr, and the raw materials may be selected and used so that the Zr content can be in the range of 0.005% by mass to 0.3% by mass. Element A may be Ti, and the raw materials may be selected and used so that the Zr content can be in the range of 0.005% by mass to 0.25% by mass. The raw materials may be selected and used so that the mole ratio of carbon to element A can be 8.4 or less. The use in such a manner of the raw materials suggests that a material having the same composition as a copper alloy will be used in the subsequent steps: the homogenization heat treatment step, the hot working step, the solution heat treatment step, and the hardening heat treatment step.

The casting may be performed by a fully continuous process, a semi-continuous process or a batch process. Alternatively, horizontal casting, vertical casting or the like may be applied. The ingot may be in the form of, for example, a slab, a billet, a bloom, a plate, a bar, a tube, or a block, and may be in any other form.

### (b) Homogenization heat treatment step

In this step, the copper alloy obtained in step (a) is heat-treated to eliminate or reduce in amount non-uniform textures, such as micro-segregates and compounds produced in nonequilibrium manner during casting, which may affect the subsequent steps, thus forming a uniform texture. The homogenization heat treatment may be performed by holding the alloy at a temperature, for example, in the range of 700°C to 1000°C, preferably 800°C to 900°C, for a period in the range of 3 hours to 24 hours, preferably 8 hours to 20 hours. In an alloy containing a large amount of Ni or Sn, the Ni or Sn is liable to segregate. The homogenization heat treatment however eliminates or reduces in amount, for example, the micro-segregates of Ni or Sn in the ingot, thus reducing the occurrence of cracks during hot working and preventing remaining non-uniform Sn enriched phases in the copper alloy from degrading the elongation and fatigue property of the alloy. For an ingot having, for example, such quality as to contain micro-segregates or dendrite arms having small distances therebetween (that is, an ingot that can produce a homogeneous texture by the subsequent solution heat treatment), the homogenization heat treatment may not be necessary.

### (c) Hot working step

In this step, the copper alloy obtained in step (a) or (b) is hot-worked into a desired shape. The hot working may be performed by, for example, hot rolling, hot extrusion, hot drawing, hot forging, or the like. These hot working methods may be combined. The hot rolling may be flat rolling using flat rolls, or other rolling, such as groove rolling using grooved rolls. The hot working may be performed at a temperature in the range of 600°C to 900°C, preferably 700°C to 900°C. The cross-section area reduction by hot working (= (cross-section area before hot working - cross-section area after hot working) / cross-section area before hot working) may be 50% or more, 70% or more, or 80% or more. If hot forging is performed as the hot working, the equivalent strain produced in the hot forging may be 0.5 or more, 3 or more, or 5 or more. The equivalent strain is defined as the sum of the absolute values of natural logarithms of the ratio of cross-section areas before and after working.

### (d) Solution heat treatment step

In this step, the copper alloy obtained in any of steps (a) to (c) is heated and then rapidly cooled to dissolve Ni, Sn and the like in Cu for forming a solid solution. The solution heat treatment may be performed by holding the alloy, for example, at a temperature in the range of 700°C to 950°C for a period in the range of 5 seconds to 6 hours, and subsequently cooling the alloy immediately and rapidly at a cooling rate of 20°C/s or more using water, oil or air. In the case of a copper alloy based on a composition of Cu-9% by mass Ni-6% by mass Sn or a composition of Cu-21% by mass Ni-5% by mass Sn, the alloy is preferably held at a temperature in the range of 750°C to 850°C for a period in the range of 5 seconds to 500 seconds (more preferably in the range of 30 seconds to 240 seconds), and then immediately cooled with water. In the case of a copper alloy based on a composition of Cu-15% by mass Ni-8% by mass Sn, the alloy is preferably held at a temperature in the range of 790°C to 870°C for a period in the range of 0.75 hour to 6 hours (more preferably in the range of 1 hour to 4 hours), and then immediately cooled with water.

### (e) Hardening heat treatment step

In this step, the copper alloy obtained in step (d) is subjected to heat treatment for spinodal decomposition and is thus hardened. The hardening heat treatment may be performed, for example, at a temperature in the range of 300°C to 500°C for a period in the range of 1 hour to 10 hours. In the case of a copper alloy based on a composition of Cu-15% by mass Ni-8% by mass Sn, the alloy may be held at a temperature in the range of 320°C to 420°C for a period in the range of 1 hour to 10 hours. In the case of a copper alloy based on a composition of Cu-9% by mass Ni-6% by mass Sn, the alloy may be held at a temperature in the range of 300°C to 450°C for a period in the range of 2 hours to 3 hours. In the case of a copper alloy based on a composition of Cu-21% by mass Ni-5% by mass Sn, the alloy may be held at a temperature in the range of 350°C to 500°C for a period in the range of 2 hours to 3 hours. If a thin plate is subjected to mill hardening heat treatment, the holding time can be shortened in each of the above cases because the thin plate has a small heat capacity.

The above-described copper alloy of the present invention is superior in ductility. Accordingly, the copper alloy can be used in, for example, articles required to have a high strength and a large elongation after fracture. Since the copper alloy exhibits satisfactory ductility at high temperatures, and is accordingly not liable to crack during hot working. Furthermore, the copper alloy that has been subjected to solution heat treatment and hardening heat treatment has high strength and exhibits high ductility and high absorbed energy of Charpy impact test, and is accordingly expected to be used in wider range of applications including an application requiring high reliability. In general, copper alloys having a large Sn content are liable to crack during hot working. In contrast, the copper alloy of the present invention is not liable to crack during hot working in spite of a relatively high Sn content. Also, in copper alloys having a large Ni content, carbon dissolved in the copper alloy can precipitate as graphite after solidification. This degrades the ductility of the copper alloy during hot working or the resulting product. Even if precipitate of graphite is not observed in the alloy, the carbon atoms that form a solid solution in the alloy may inhibit the migration of dislocation when the material is plastically deformed, and thus degrade the ductility of the copper alloy during hot working or the resulting produce. In contrast, the copper alloy of the present invention exhibits satisfactory ductility during hot working or in the resulting product in spite of a relatively high Ni content.

Furthermore, since the copper alloy of the present invention is superior in ductility and good in workability during hot working or cold working, wide varieties of manufacturing methods and intended product shapes can be applied. Known Cu-Ni-Sn-based copper alloys, of which the hot working is difficult, are casted into plates by a horizontal continuous casting process capable of casting with dimensions relatively close to the intended product dimensions, and then the plates are worked into articles in a strip shape, such as thin plates, through repetitions of cold rolling and annealing. On the other hand, the copper alloy having the composition according to the present invention is superior in ductility and is not liable to crack during hot forging or hot rolling of the ingot. The copper alloy of the present invention can therefore be relatively easily worked into dimensions or a shape relatively close to the dimensions or shape of the intended product. Thus, casting methods other than horizontal continuous casting can be applied irrespective of the dimensions or shape of the ingot. The known horizontal continuous casting does not cause a large problem in large-lot mass production. In the case of small-lot production, however, molten metal tends to remain in the horizontal melting holding furnace and results in a reduced yield. The copper alloy of the present invention however can be casted by, for example, vertical continuous casting and can be casted in a small lot production with a high yield, accordingly being suitable for semi-continuous casting as well as fully continuous casting. Since vertical continuous casting can be applied, round ingots and rectangular ingots can be easily produced. Such a round ingot or rectangular ingot can be easily forged into a product in a block or billet shape having a large cross section with an aspect ratio close to 1. Also, the copper alloy of the present invention is good in workability in hot rolling or cold rolling and can be worked into products in various shapes. Accordingly, the copper alloy is expected to be used for products other than thin plates and strips.

The copper alloy of the present invention, which is a Cu-Ni-Sn-based copper alloy having a high strength and a low friction coefficient, can be suitably used for sliding members, such as bearings, and structural members such as bars, tubes and blocks. The copper alloy is suitable for use as conductive members, such as wires, leaf springs (thin plate strip materials) of connectors or the like because of high strength, electric conductivity and bending formability thereof. Furthermore, the copper alloy is superior in stress relaxation characteristic and is accordingly suitable for use as terminal members such as burn-in socket, relay terminals, or springs that are used in high-temperature environment.

The present invention is not limited to the above-described embodiment, and it should be appreciated that various forms can be applied to the invention within the technical scope of the invention.

For example, the copper alloy of the above-described embodiment is prepared in a manufacturing process including steps (a) to (e). The process is not limited to this. For example, the process may consist of step (a), omitting steps (b) to (e). The As-cast material produced through such a process is suitably used in steps (b) to (e) and the like, and has good workability and can provide a highly ductile and strong article. The manufacturing process may omit steps (c) to (e), step (d) and (e), or step (e). The resulting material produced through such a process is suitably used in the operation of the omitted step or the like.

The manufacturing process of the copper alloy may further include a cold working step between steps (d) and (e). The cold working may be performed by, for example, cold rolling, cold extrusion, cold drawing, cold forging, or the like. These cold working methods may be combined. The cold working step may be substituted for step (c), or may be performed between steps (c) and (d). In this instance, the cold working step and an annealing step may be repeated. The cold working may be performed by any one of the above-mentioned methods.

### EXAMPLES

Specific examples of the copper alloy will now be described as Experimental Examples. Experimental Examples 3, 4, 6, 8 to 16, 18, 20, and 21 correspond to Examples of the present invention, and Experiment Examples 1, 2, 5, 7, 17, and 19 correspond to Comparative Examples. The present invention is not limited to the following Experimental Examples, and it should be appreciated that various forms can be applied to the invention within the technical scope of the invention.

### [Experimental Examples 1 to 16]

### (Preparation of Copper Alloy)

Raw materials including electrolytic copper, electrolytic nickel, tin and 35% by mass Mn-Cu alloy were melted in a graphite or ceramic crucible in an argon atmosphere in a high-frequency induction melting furnace to yield a 110 mm in diameter by 200 mm ingot of Cu-15% by mass Ni-8% by mass Sn-0.2% by mass Mn alloy containing additive elements shown in Table 2. The Nb source was 60% by mass Nb-Ni; the Zr source was metallic Zr; and the Ti source was metallic Ti. As a carbon source, a graphite-containing covering material for molten metal was optionally used. The carbon content was controlled by varying the type and amount of the covering material added to the molten metal, the contact time between the molten metal and the covering material, or the temperature at which the molten metal was held. The amounts of element A shown in the Tables were values measured by a wet chemical analysis (ICP), and the amounts of carbon in the Tables were values measured by a infrared absorption method after combustion in oxygen flow with a carbon analyzer.

After being held at 900°C for 8 hours for homogenization heat treatment, the ingot was cut into a 42 mm in diameter × 95 mm round bar as a material for hot rolling with grooved rolls. The round bar was heated to 850°C and then rolled into a rectangular bar with a cross section of about 16 mm × 16 mm by the rolling. The states of cracks that occurred after the rolling are shown in Table 2. The state of cracks were evaluated according to the following: samples that fractured while the sample is under the rolling or machining were rated as "fractured"; samples in which five or more cracks of 3 mm or more in depth occurred within a length of 100 mm were rated as "large"; samples in which one to four cracks of 3 mm or more in depth occurred within a length of 100 mm were rated as "rather large"; samples in which five or more cracks of less than 3 mm in depth occurred within a length of 100 mm whereas cracks of 3 mm or more in depth did not occur were rated as "middle"; and samples in which four or less cracks of less than 3 mm in depth occurred within a length of 100 mm whereas cracks of 3 mm or more in depth did not occur were rated as "small". For reference, Fig. 1 shows appearance photographs of samples after being subjected to the rolling in Experimental Examples 2, 4, 9 and 12.

After being heated at 830°C for 2 hours, the groove-rolled bar was immediately cooled in water for solution treatment, and then subjected to hardening heat treatment at 370°C for 4 hours. The resulting rectangular bar was worked into a specimen for tensile test, and the specimen was subjected to tensile test (according to JIS Z 2241, the same applies hereinafter) at room temperature. The results of the tensile test are shown in Table 2.

### (Experiment Results and Consideration)

In Experimental Examples 1 and 2, in which element A was not added, cracks occurred markedly during the hot rolling with grooved rolls. Consequently, the samples were not worked into specimens for tensile test, or the specimens exhibited very small elongation in the tensile test. In Experimental Examples 3 to 16, in which element A was added, cracks that occurred during the hot rolling were smaller than in Experimental Examples 1 and 2, and elongation was larger in the tensile test.

In Experimental Examples 3 to 6, 13, and 14, Nb was added as element A. Among these Experimental Examples, Experimental Examples 3, 4, 6, 13, and 14, containing 0.005% by mass or more of carbon exhibited larger elongation and higher tensile strength than Experimental Example 5 containing 0.002% by mass of carbon. These results reversed the common perception that Cu alloys containing a relatively large amount of Ni tend to have a lower ductility (becomes brittler) as the carbon content is increased. In the observation of microstructure of Experimental Examples 1 to 6, many phases (having a grain size of the phase about 3 µm to 5 µm, for large grains) that were assumed to be Nb carbide were observed in Experimental Examples 3, 4 and 6. On the other hand, in Experimental Examples 1, 2 and 5, there were observed no phases or few phases that were assumed to be carbide. Fig. 2 shows an electron micrograph (COMPO image, the same applies hereinafter) and EPMA analysis results (characteristic X-ray images of carbon and niobium) of the ingot of Experimental Example 6. The white granular phase in the COMPO image was observed at the same position as the white portions in the characteristic X-ray images representing the presence of carbon or niobium. This suggests that the white phase is a Nb carbide phase. The average grain sizes of the microstructure after being subjected to hardening heat treatment in Experimental Examples 4, 5 and 6 were measured by the intercept procedure specified in ASTM E112. The results were 45 µm, 211 µm and 115 µm, respectively. From these results, it is assumed that, in copper alloys containing appropriate amounts of Nb and carbon, elemental carbon that is the cause of decrease in ductility (becoming brittle) is reduced in amount by being used for the formation of the Nb carbide, and that the pinning effect of the Nb carbide allows the crystal grains to become finer and thus increases elongation and tensile strength.

In Experimental Examples 7 to 11, 15, and 16, Zr was added as element A. Among these Experimental Examples, Experimental Examples 8 to 11, 15, and 16 with a MC/MA mole ratio of 10.0 or less exhibited larger elongation and higher tensile strength than Experimental Example 7 with a MC/MA mole ratio of 10.3. Also, Experimental Example 9 having a higher carbon content than Experimental Example 7 exhibited larger elongation and higher tensile strength than Experimental Example 7. These results suggest that the upper limit of the carbon content varies depending on the element A content. It is assumed that the elongation of a sample with a large MC/MA mole ratio is small because of the presence of an excessively large amount of carbon not forming Zr carbide. Fig. 3 shows electron micrographs and EPMA mapping results of the microstructure of the ingot of Experimental Example 9. Fig. 4 shows electron micrographs and EPMA mapping results of the copper alloy after being subjected to hardening heat treatment in Experimental Example 8. In the EPMA mapping results shown in Figs. 3 and 4, the images denoted by CP are COMPO images at positions of mapping performed, and images denoted by Zr, Cu, C, Ni, or Sn are EPMA mapping images of the corresponding element. The higher content of the corresponding element, is the whiter mapping image, which is originally a color image. In portions in the EPMA mapping images corresponding to the angulated phases in the COMPO images, larger amounts of carbon and Zr were observed, while Cu, Ni and Sn were smaller in amount. These results suggest that the angulated phases were Zr carbide phases. The phases that were assumed to be Zr carbide phases were further subjected to composition analysis (at three points for each) using a COMPO image (× 3000). The results are shown in Table 1. As shown in Table 1, the mole ratio of Zr to carbon in the angulated phases was about 1:1, and this suggests that the phases were of ZrC. The average grain size of the microstructure after being subjected to hardening heat treatment in Experimental Example 8, measured by the intercept procedure specified in ASTM E112, was 48 µm. Similarly, the average grain sizes of the microstructure after being subjected to hardening heat treatment in Experimental Examples 9 and 11, measured in the same manner, were each 35 µm. From these results, it is assumed that, in copper alloys containing appropriate amounts of Zr and carbon, elemental carbon that is the cause of decrease in ductility (becoming brittle) is reduced in amount by being used for the formation of carbide with the Zr, and that the effect of the Zr carbide to pin dislocation allows the crystal grains to become finer and thus increases elongation and tensile strength. For the sake of comparison, Fig. 5 shows an electron micrograph and EPMA mapping images of Experimental Example 2. Fig. 5 suggests that samples not containing element A causes carbon to precipitate, and that such a microstructure reduces ductility.

**Table 1**

| Ingot (Experimental Example 9) | | | | After being subjected to hardening heat treatment (Experimental Example 8) | | | |
|---|---|---|---|---|---|---|---|
| No | C | Zr | Total | No | C | Zr | Total |
| | Atomic % | Atomic % | Atomic % | | Atomic % | Atomic % | Atomic % |
| Average | 45.7 | 54.3 | 100.0 | Average | 46.7 | 53.3 | 100.0 |
| 1 | 45.5 | 54.5 | 100.0 | 4 | 48.2 | 51.8 | 100.0 |
| 2 | 46.4 | 53.6 | 100.0 | 5 | 46.2 | 53.8 | 100.0 |
| 3 | 45.1 | 54.9 | 100.0 | 6 | 45.6 | 54.4 | 100.0 |

In Experimental Example 12, Ti was added as element A. The elongation and tensile strength of this Example were also large. From these results, it is assumed that, in copper alloys containing appropriate amounts of Ti and carbon, elemental carbon that is the cause of decrease in ductility (becoming brittle) is reduced in amount by being used for the formation of carbide with the Ti, and that the pinning effect of the Ti carbide allows the crystal grains to become finer and thus increases elongation and tensile strength.

**Table 2**

| | Additive elements | | | | | Evaluation | | |
|---|---|---|---|---|---|---|---|---|
| | Element A | | | C | Mole ratio MC/MA | Cracks occurred after rolling with grooved rolls | Tensile strength | Elongation |
| | Nb | Zr | Ti | | | | | |
| | mass% | mass% | mass% | mass% | - | - | MPa | % |
| Experimental Example 1 | Not added | Not added | Not added | 0.003 | - | Large | 755 | 1.2 |
| Experimental Example 2 | Not added | Not added | Not added | 0.018 | - | Fractured | Specimen could not be prepared | |
| Experimental Example 3 | 0.015 | Not added | Not added | 0.007 | 3.6 | Small | 915 | 15.0 |
| Experimental Example 4 | 0.040 | Not added | Not added | 0.020 | 3.9 | Middle | 949 | 19.2 |
| Experimental Example 5 | 0.050 | Not added | Not added | 0.002 | 0.3 | Large | 848 | 4.9 |
| Experimental Example 6 | 0.085 | Not added | Not added | 0.021 | 1.9 | Middle | 936 | 15.3 |
| Experimental Example 7 | Not added | 0.036 | Not added | 0.049 | 10.3 | Large | 910 | 4.5 |
| Experimental Example 8 | Not added | 0.078 | Not added | 0.013 | 1.3 | Small | 954 | 15.1 |
| Experimental Example 9 | Not added | 0.084 | Not added | 0.058 | 5.2 | Small | 946 | 25.0 |
| Experimental Example 10 | Not added | 0.184 | Not added | 0.010 | 0.4 | Small | 972 | 17.0 |
| Experimental Example 11 | Not added | 0.278 | Not added | 0.009 | 0.2 | Middle | 964 | 19.3 |
| Experimental Example 12 | Not added | Not added | 0.080 | 0.031 | 1.5 | Small | 916 | 12.5 |
| Experimental Example 13 | 0.021 | Not added | Not added | 0.018 | 6.6 | Middle | 940 | 15.1 |
| Experimental Example 14 | 0.013 | Not added | Not added | 0.014 | 8.3 | Middle | 924 | 10.5 |
| Experimental Example 15 | Not added | 0.085 | Not added | 0.072 | 6.4 | Small | 938 | 21.8 |
| Experimental Example 16 | Not added | 0.069 | Not added | 0.076 | 8.4 | Small | 943 | 14.5 |

Note that Experimental Examples 1, 2, 5 and 7 are outside the scope of the invention.

### [Experimental Examples 17 and 18]

### (Preparation of Copper Alloy)

Raw materials including electrolytic copper, electrolytic nickel, tin and 35% by mass Mn-Cu alloy were melted in a graphite crucible in an argon atmosphere in a high-frequency induction melting furnace to yield an ingot of Cu-15% by mass Ni-8% by mass Sn-0.2% by mass Mn alloy containing additive elements shown in Table 3. The sound part of the ingot measured 275 mm in diameter × 500 mm. The Nb source was 60% by mass Nb-Ni alloy. The carbon source was the graphite crucible, and the carbon content was adjusted by controlling the contact time between the graphite crucible and the molten metal or the time at which the molten metal was held.

After being held at 900°C for 8 hours for homogenization heat treatment, the ingot was turned at the surface and was hot-extruded into a round bar of about 100 mm in diameter at 850°C. After being heated at 830°C for 2 hours, the round bar was immediately cooled in water for solution treatment, and then subjected to hardening heat treatment at 370°C for 4 hours. The resulting round bar was worked into a specimen for tensile test, and the specimen was subjected to tensile test at room temperature. The results of the tensile test are shown in Table 3.

### (Experiment Results and Discussion)

Experimental Example 18, in which element A was added, exhibited a lager elongation in the tensile test than the Experimental Example 17, in which element A was not added. Experimental Example 18 also exhibited a high tensile strength as a whole.

**Table 3**

| | Additive elements | | | | Evaluation | | |
|---|---|---|---|---|---|---|---|
| | Element A | | C | Mole ratio MC/MA | Position where the specimen was obtained | Tensile strength | Elongation |
| | Nb | Zr | | | | | |
| | mass% | mass% | mass% | - | - | MPa | % |
| Experimental Example 17 | Not added | Not added | 0.010 | - | Center of nose portion | 916 | 5.5 |
| | | | | | Peripheral of nose portion | 908 | 4.1 |
| | | | | | Center of near butt-end portion | 918 | 8.9 |
| | | | | | Peripheral of near butt-end portion | 930 | 6.7 |
| Experimental Example 18 | 0.026 | Not added | 0.015 | 4.5 | Center of nose portion | 924 | 11.1 |
| | | | | | Peripheral of nose portion | 955 | 12.7 |
| | | | | | Center of near butt-end portion | 929 | 14.1 |
| | | | | | Peripheral of near butt-end portion | 948 | 15.5 |

### [Experimental Examples 19 to 21]

Raw materials including electrolytic copper, electrolytic nickel, tin and 35% by mass Mn-Cu alloy were melted in a graphite crucible in an argon atmosphere in a high-frequency induction melting furnace to yield an ingot of Cu-15% by mass Ni-8% by mass Sn-0.2% by mass Mn alloy containing additive elements shown in Table 4. The sound part of the ingot measured 275 mm in diameter × 380 mm. The Nb source was 60% by mass Nb-Ni alloy, and the Zr source was metallic Zr. The carbon source was the same graphite crucible as in Experimental Examples 17 and 18.

The ingot, surface of which was turned was held at 900°C for 8 hours for homogenization heat treatment and was then cooled to 850°C. The sample was subjected to hot forging for an intended round bar of about 180 mm in diameter × 600 mm with an equivalent strain of 6.

In Experimental Example 19, in which element A was not added, a plurality of large cracks occurred in the side surfaces at the time when upsetting was performed with an equivalent strain of 0.7. Therefore the subsequent forging was canceled. In Experimental Examples 20 and 21, in which element A was added, upsetting and forging were alternately repeated to an equivalent strain of 6 while relative small creases and cracks in the surface were removed by grinding. In Experimental Example 20, a crack that could be removed by cutting occurred in one end of the round bar during the final forging operation. In Experimental Example 21, forging was completed without occurrence of marked cracks. Figs. 6 to 8 show the appearances of forged products of Experimental Examples 19 to 21. It was thus confirmed that the copper alloy of the present invention can be subjected to hot forging and relatively easily worked into various shapes. Accordingly, the copper alloy is expected to be used in a wide range of applications.

**Table 4**

| | Additive elements | | | | Evaluation |
|---|---|---|---|---|---|
| | Element A | | C | Mole ratio MC/MA | Equivalent strain (target value: 6) |
| | Nb | Zr | | | |
| | mass% | mass% | mass% | - | - |
| Experimental Example 19 | Not added | Not added | 0.012 | - | 0.7 |
| Experimental Example 20 | 0.072 | Not added | 0.013 | 1.4 | 6 |
| Experimental Example 21 | Not added | 0.099 | 0.011 | 0.8 | 6 |

| | | | | | |
|---|---|---|---|---|---|
| Relative small creases and cracks occurred in the surface, but the forging was operated while cracks were removed by grinding | | | | | |

### Industrial Applicability

The present invention can be applied to the field related to copper alloy.

## Claims

1. A copper alloy consisting of:
5% by mass to 25% by mass of Ni;
5% by mass to 10% by mass of Sn;
0.005% by mass to 0.5% by mass of element A, element A being at least one selected from the group consisting of Nb, Zr and Ti;
0.005% by mass or more of carbon, wherein the mole ratio of the carbon to the element A is 10.0 or less;
optionally, 0.01% by mass to 1% by mass of an additive element, the additive element being at least one selected from the group consisting of Mn, Zn, Mg, Ca, Al, Si, P, and B, and
the balance of the composition of the copper alloy is Cu and inevitable impurities.

2. The copper alloy according to Claim 1, wherein 0.01% by mass to 1% by mass of the additive element, the additive element being at least one selected from the group consisting of Mn, Zn, Mg, Ca, Al, Si, P, and B, is present.

3. The copper alloy according to Claim 1 or 2, containing 14.0% by mass to 16.0% by mass of Ni, and 7.0% by mass to 9.0% by mass of Sn.

4. The copper alloy according to any one of Claims 1 to 3, wherein the element A is Nb, and containing 0.005% by mass to 0.1% by mass of Nb.

5. The copper alloy according to any one of Claims 1 to 3, wherein the element A is Zr, and containing 0.005% by mass to 0.3% by mass of Zr.

6. The copper alloy according to any one of Claims 1 to 3, wherein the element A is Ti, and containing 0.005% by mass to 0.25% by mass of Ti.

7. The copper alloy according to any one of Claims 1 to 6, wherein at least part of the element A is present as carbide.

8. The copper alloy according to any one of Claims 1 to 7, wherein the mole ratio of carbon to the element A is 8.4 or less.

9. The copper alloy according to any one of Claims 1 to 8, wherein the copper alloy exhibits an elongation after fracture of 10% or more.

10. The copper alloy according to any one of Claims 1 to 9, wherein the copper alloy has a tensile strength of 915 MPa or more.

11. A method for manufacturing a copper alloy, the method comprising:
a melting and casting step of melting and casting raw materials consisting of:
5% by mass to 25% by mass of Ni;
5% by mass to 10% by mass of Sn;
0.005% by mass to 0.5% by mass of element A, element A being at least one selected from the group consisting of Nb, Zr and Ti;
0.005% by mass or more of carbon, wherein the mole ratio of the carbon to the element A is 10.0 or less;
optionally, 0.01% by mass to 1% by mass of an additive element, the additive element being at least one selected from the group consisting of Mn, Zn, Mg, Ca, Al, Si, P, and B, and
the balance of the composition of the raw materials consists of Cu and inevitable impurities.

12. The method for manufacturing a copper alloy according to Claim 11, the method further comprising:
a homogenization heat treatment step of applying homogenization heat treatment at a temperature in the range of 700°C to 1000°C for a period in the range of 3 hours to 10 hours to the copper alloy that has been subjected to the melting and casting step.

13. The method for manufacturing a copper alloy according to Claim 11 or 12, the method further comprising:
a solution heat treatment step of heating at a temperature of 700°C or more the copper alloy that has been subjected to the melting and casting step, and then cooling the copper alloy rapidly at a rate of 20°C/s or more, thereby forming a solid solution.

14. The method for manufacturing a copper alloy according to any one of Claims 11 to 13, the method further comprising:
a hardening heat treatment step of heat-treating the copper alloy that has been subjected to the melting and casting step to cause spinodal decomposition, thereby hardening the copper alloy.

15. The method for manufacturing a copper alloy according to any one of Claims 11 to 14, wherein in the melting and casting step, the raw materials contain said 0.01% by mass to 1% by mass of the additive element, being at least one selected from the group consisting of Mn, Zn, Mg, Ca, Al, Si, P, and B.

16. The method for manufacturing a copper alloy according to any one of Claims 11 to 15, in the melting and casting step, using the raw materials containing 14.0% by mass to 16.0% by mass of Ni, and 7.0% by mass to 9.0% by mass of Sn.

17. The method for manufacturing a copper alloy according to any one of Claims 11 to 16, in the melting and casting step, using the raw materials wherein the element A is Nb and containing 0.005% by mass to 0.1% by mass of Nb.

18. The method for manufacturing a copper alloy according to any one of Claims 11 to 16, in the melting and casting step, using the raw materials wherein the element A is Zr and containing 0.005% by mass to 0.3% by mass of Zr.

19. The method for manufacturing a copper alloy according to any one of Claims 11 to 16, in the melting and casting step, using the raw materials wherein the element A is Ti and containing 0.005% by mass to 0.25% by mass of Ti.

20. The method for manufacturing a copper alloy according to any one of Claims 11 to 19, in the melting and casting step, using the raw materials having the mole ratio of carbon to the element A being 8.4 or less.

## Patentansprüche

1. Kupferlegierung, bestehend aus:
5 Masse-% bis 25 Masse-% Ni;
5 Masse-% bis 10 Masse-% Sn;
0,005 Masse-% bis 0,5 Masse-% eines Elements A, wobei Element A zumindest ein aus der aus Nb, Zr und Ti bestehenden Gruppe ausgewähltes Element ist;
0,005 Masse-% oder mehr Kohlenstoff, wobei das Molverhältnis des Kohlenstoffs zu Element A 10,0 oder weniger beträgt;
gegebenenfalls 0,01 Masse-% bis 1 Masse-% eines Zusatzelements, wobei das Zusatzelements zumindest ein aus der aus Mn, Zn, Mg, Ca, Al, Si, P und B bestehenden Gruppe ausgewähltes Element ist; und
der Rest der Zusammensetzung der Kupferlegierung Cu und unvermeidbare Verunreinigungen ist.

2. Kupferlegierung nach Anspruch 1, wobei 0,01 Masse-% bis 1 Masse-% des Zusatzelements vorliegen, wobei das Zusatzelement zumindest ein aus der aus Mn, Zn, Mg, Ca, Al, Si, P und B bestehenden Gruppe ausgewähltes Element ist.

3. Kupferlegierung nach Anspruch 1 oder 2, die 14,0 Masse-% bis 16,0 Masse-% Ni und 7,0 Masse-% bis 9,0 Masse-% Sn enthält.

4. Kupferlegierung nach einem der Ansprüche 1 bis 3, wobei Element A Nb ist und 0,005 Masse-% bis 0,1 Masse-% Nb enthalten sind.

5. Kupferlegierung nach einem der Ansprüche 1 bis 3, wobei Element A Zr ist und 0,005 Masse-% bis 0,3 Masse-% Zr enthalten sind.

6. Kupferlegierung nach einem der Ansprüche 1 bis 3, wobei Element A Ti ist und 0,005 Masse-% bis 0,25 Masse-% Ti enthalten sind.

7. Kupferlegierung nach einem der Ansprüche 1 bis 6, wobei zumindest ein Teil von Element A als Carbid vorliegt.

8. Kupferlegierung nach einem der Ansprüche 1 bis 7, wobei das Molverhältnis von Kohlenstoff zu Element A 8,4 oder weniger beträgt.

9. Kupferlegierung nach einem der Ansprüche 1 bis 8, wobei die Kupferlegierung eine Bruchdehnung von 10 % oder mehr aufweist.

10. Kupferlegierung nach einem der Ansprüche 1 bis 9, wobei die Kupferlegierung eine Zugfestigkeit von 915 MPa oder mehr aufweist.

11. Verfahren zur Herstellung einer Kupferlegierung, wobei das Verfahren Folgendes umfasst:
einen Schmelz- und Gießschritt des Schmelzens und Gießens von Rohmaterialien, die aus Folgendem bestehen:
5 Masse-% bis 25 Masse-% Ni;
5 Masse-% bis 10 Masse-% Sn;
0,005 Masse-% bis 0,5 Masse-% von Element A, wobei Element A zumindest ein aus der aus Nb, Zr und Ti bestehenden Gruppe ausgewähltes Element ist;
0,005 Masse-% oder mehr Kohlenstoff, wobei das Molverhältnis des Kohlenstoffs zu Element A 10,0 oder weniger beträgt;
gegebenenfalls 0,01 Masse-% bis 1 Masse-% eines Zusatzelements, wobei das Zusatzelements zumindest ein aus der aus Mn, Zn, Mg, Ca, Al, Si, P und B bestehenden Gruppe ausgewähltes Element ist; und
der Rest der Zusammensetzung der Rohmaterialien aus Cu und unvermeidbaren Verunreinigungen besteht.

12. Verfahren zur Herstellung einer Kupferlegierung nach Anspruch 11, wobei das Verfahren weiters Folgendes umfasst:
einen Homogenisierungswärmebehandlungsschritt, bei dem die dem Schmelz- und Gießschritt unterzogene Kupferlegierung einer Homogenisierungswärmebehandlung bei einer Temperatur im Bereich von 700 °C bis 1000 °C für einen Zeitraum im Bereich von 3 Stunden bis 10 Stunden unterzogen wird.

13. Verfahren zur Herstellung einer Kupferlegierung nach Anspruch 11 oder 12, wobei das Verfahren weiters Folgendes umfasst:
einen Lösungswärmebehandlungsschritt, bei dem die dem Schmelz- und Gießschritt unterzogene Kupferlegierung auf eine Temperatur von 700 °C oder mehr erhitzt wird und die Kupferlegierung dann mit einer Rate von 20 °C/s oder mehr rasch abgekühlt wird, wodurch eine feste Lösung ausgebildet wird.

14. Verfahren zur Herstellung einer Kupferlegierung nach einem der Ansprüche 11 bis 13, wobei das Verfahren weiters Folgendes umfasst:
einen Härtungswärmebehandlungsschritt, bei dem die dem Schmelz- und Gießschritt unterzogene Kupferlegierung einer Wärmebehandlung unterzogen wird, um eine spinodale Auflösung zu verursachen, wodurch die Kupferlegierung gehärtet wird.

15. Verfahren zur Herstellung einer Kupferlegierung nach einem der Ansprüche 11 bis 14, wobei die Rohmaterialien im Schmelz- und Gießschritt 0,01 Masse-% bis 1 Masse-% des Zusatzelements enthalten, das zumindest ein aus der aus Mn, Zn, Mg, Ca, Al, Si, P und B bestehenden Gruppe ausgewähltes Element ist.

16. Verfahren zur Herstellung einer Kupferlegierung nach einem der Ansprüche 11 bis 15, wobei im Schmelz- und Gießschritt Rohmaterialien verwendet werden, die 14,0 Masse-% bis 16,0 Masse-% Ni und 7,0 Masse-% bis 9,0 Masse-% Sn enthalten.

17. Verfahren zur Herstellung einer Kupferlegierung nach einem der Ansprüche 11 bis 16, wobei im Schmelz- und Gießschritt Rohmaterialien verwendet werden, von denen Element A Nb ist und 0,005 Masse-% bis 0,1 Masse-% Nb enthalten sind.

18. Verfahren zur Herstellung einer Kupferlegierung nach einem der Ansprüche 11 bis 16, wobei im Schmelz- und Gießschritt Rohmaterialien verwendet werden, von denen Element A Zr ist und 0,005 Masse-% bis 0,3 Masse-% Zr enthalten sind.

19. Verfahren zur Herstellung einer Kupferlegierung nach einem der Ansprüche 11 bis 16, wobei im Schmelz- und Gießschritt Rohmaterialien verwendet werden, von denen Element A Ti ist und 0,005 Masse-% bis 0,25 Masse-% Ti enthalten sind.

20. Verfahren zur Herstellung einer Kupferlegierung nach einem der Ansprüche 11 bis 19, wobei im Schmelz- und Gießschritt Rohmaterialien mit einem Molverhältnis von Kohlenstoff zu Element A von 8,4 oder weniger verwendet werden.

## Revendications

1. Alliage de cuivre constitué par :
de 5 % en masse à 25 % en masse de Ni ;
de 5 % en masse à 10 % en masse de Sn ;
de 0,005 % en masse à 0,5 % en masse de l'élément A, l'élément A étant au moins choisi dans le groupe constitué par Nb, Zr et Ti ;
0,005 % en masse ou plus de carbone, le rapport molaire du carbone à l'élément A étant inférieur ou égal à 10,0 ;
facultativement, de 0,01 % en masse à 1 % en masse d'un élément additif, l'élément additif étant au moins choisi dans le groupe constitué par Mn, Zn, Mg, Ca, Al, Si, P et B, et
le reste de la composition de l'alliage de cuivre étant du Cu et des impuretés inévitables.

2. Alliage de cuivre selon la revendication 1, dans lequel est présent de 0,01 % en masse à 1 % en masse de l'élément additif, l'élément additif étant au moins un élément choisi dans le groupe constitué par Mn, Zn, Mg, Ca, Al, Si, P et B.

3. Alliage de cuivre selon la revendication 1 ou 2, contenant de 14,0 % en masse à 16,0 % en masse de Ni, et de 7,0 % en masse à 9,0 % en masse de Sn.

4. Alliage de cuivre selon l'une quelconque des revendications 1 à 3, dans lequel l'élément A est le Nb, et contenant de 0,005 % en masse à 0,1 % en masse de Nb.

5. Alliage de cuivre selon l'une quelconque des revendications 1 à 3, dans lequel l'élément A est le Zr, et contenant de 0,005 % en masse à 0,3 % en masse de Zr.

6. Alliage de cuivre selon l'une quelconque des revendications 1 à 3, dans lequel l'élément A est le Ti, et contenant de 0,005 % en masse à 0,25 % en masse de Ti.

7. Alliage de cuivre selon l'une quelconque des revendications 1 à 6, dans lequel au moins une partie de l'élément A est présente sous forme de carbure.

8. Alliage de cuivre selon l'une quelconque des revendications 1 à 7, dans lequel le rapport molaire du carbone à l'élément A est inférieur ou égal à 8,4.

9. Alliage de cuivre selon l'une quelconque des revendications 1 à 8, dans lequel l'alliage de cuivre présente un allongement après fracture supérieur ou égal à 10 %.

10. Alliage de cuivre selon l'une quelconque des revendications 1 à 9, dans lequel l'alliage de cuivre a une résistance à la traction supérieure ou égale à 915 MPa.

11. Procédé de fabrication d'un alliage de cuivre, le procédé comprenant :
une étape de fusion et de coulage consistant à faire fondre et couler les matières premières constituées par :
de 5 % en masse à 25 % en masse de Ni ;
de 5 % en masse à 10 % en masse de Sn ;
de 0,005 % en masse à 0,5 % en masse de l'élément A, l'élément A étant au moins choisi dans le groupe constitué par Nb, Zr et Ti ;
0,005 % en masse ou plus de carbone, le rapport molaire du carbone à l'élément A étant inférieur ou égal à 10,0 ;
facultativement, de 0,01 % en masse à 1 % en masse d'un élément additif, l'élément additif étant au moins choisi dans le groupe constitué par Mn, Zn, Mg, Ca, Al, Si, P et B, et
le reste de la composition des matières premières se composant de Cu et d'impuretés inévitables.

12. Procédé de fabrication d'un alliage de cuivre selon la revendication 11, le procédé comprenant en outre :
une étape de traitement thermique d'homogénéisation consistant à appliquer un traitement thermique d'homogénéisation à une température comprise dans la plage allant de 700 °C à 1 000 °C pendant une période comprise dans la plage allant de 3 heures à 10 heures sur l'alliage de cuivre qui a été soumis à l'étape de fusion et coulage.

13. Procédé de fabrication d'un alliage de cuivre selon la revendication 11 ou 12, le procédé comprenant en outre :
une étape de traitement thermique en solution consistant à chauffer à une température supérieure ou égale à 700 °C l'alliage de cuivre qui a été soumis à l'étape de fusion et coulage, et ensuite à refroidir l'alliage de cuivre rapidement à une vitesse supérieure ou égale à 20 °C/s, formant ainsi une solution solide.

14. Procédé de fabrication d'un alliage de cuivre selon l'une quelconque des revendications 11 à 13, le procédé comprenant en outre :
une étape de traitement thermique de durcissement consistant à traiter thermiquement l'alliage de cuivre qui a été soumis à l'étape de fusion et coulage pour provoquer une décomposition spinodale, durcissant ainsi l'alliage de cuivre.

15. Procédé de fabrication d'un alliage de cuivre selon l'une quelconque des revendications 11 à 14, dans lequel dans l'étape de fusion et coulage, les matières premières contiennent de 0,01 % en masse à 1 % en masse dudit élément additif, qui est au moins un élément choisi dans le groupe constitué par Mn, Zn, Mg, Ca, Al, Si, P et B.

16. Procédé de fabrication d'un alliage de cuivre selon l'une quelconque des revendications 11 à 15, utilisant, dans l'étape de fusion et coulage, les matières premières contenant de 14,0 % en masse à 16,0 % en masse de Ni, et de 7,0 % en masse à 9,0 % en masse de Sn.

17. Procédé de fabrication d'un alliage de cuivre selon l'une quelconque des revendications 11 à 16, utilisant, dans l'étape de fusion et coulage, les matières premières dans lesquelles l'élément A est le Nb et contenant de 0,005 % en masse à 0,1 % en masse de Nb.

18. Procédé de fabrication d'un alliage de cuivre selon l'une quelconque des revendications 11 à 16, utilisant, dans l'étape de fusion et coulage, les matières premières dans lesquelles l'élément A est le Zr et contenant de 0,005 % en masse à 0,3 % en masse de Zr.

19. Procédé de fabrication d'un alliage de cuivre selon l'une quelconque des revendications 11 à 16, utilisant, dans l'étape de fusion et coulage, les matières premières dans lesquelles l'élément A est le Ti et contenant de 0,005 % en masse à 0,25 % en masse de Ti.

20. Procédé de fabrication d'un alliage de cuivre selon l'une quelconque des revendications 11 à 19, utilisant, dans l'étape de fusion et coulage, les matières premières ayant le rapport molaire du carbone à l'élément A qui est inférieur ou égal à 8,4.
